

Feb. 16, 1971

B. BRAUN

3,562,820

TUBULAR SHEET AND STRIP FORM PROSTHESES ON  
A BASIS OF BIOLOGICAL TISSUE  
Filed Aug. 21, 1967

FIG. 1.



FIG. 2.



FIG. 3.



FIG. 4.

INVENTOR  
BERNHARD BRAUN  
BY: *Burgess, Linkletter & Sprague*

ATTORNEYS.

## 1

3,562,820  
**TUBULAR SHEET AND STRIP FORM PROSTHESES  
ON A BASIS OF BIOLOGICAL TISSUE**  
Bernhard Braun, Trankelucke 1,  
Melsungen, Germany  
Filed Aug. 21, 1967, Ser. No. 661,900  
Claims priority, application Austria, Aug. 22, 1966,  
A 7,958/66  
Int. Cl. A61f 1/24

U.S. Cl. 3—1

5 Claims

### ABSTRACT OF THE DISCLOSURE

There are disclosed tubular, sheet and strip form prostheses on a basis of biological tissue for use in the replacement, repair and strengthening of various living organs such as the vasculature, esophagus, bronchus, intestine, ureter, liver, kidney, etc., and a process for making and using the same. The prosthesis itself comprises a unitary structure of alternating layers of natural tissue and collagen fibres. The same is manufactured by applying a strip, sheet or tube of biological material onto a substantially rigid support, coating the exposed surface with a binder paste, as for example, a collagen fibre paste, or bringing about the swelling of the exposed surface, thereafter applying a second layer of natural material and repeating the procedure until the desired wall thickness is obtained. The multi-layer prosthesis is then dried and removed from the underlying support.

The invention described herein relates to tubular, strip and sheet form prostheses on a basis of biological tissue and to methods for manufacturing and using the same. More particularly this invention relates to a multi-layer prosthesis on a basis of biological tissue.

The prostheses of the invention are suitable for use as vascular, esophagus, bronchus, intestinal, ureter and cardiac valve prostheses and as other corrective parts of various organs such as liver.

It is already known to prepare tubes and fabrics from polytetrafluoroethylene or polyester fibers, either by weaving or knitting or by a combined weaving and knitting process and to use the same to replace diseased blood vessels or parts of the heart. At first, clinical results with these prostheses were satisfactory and highly promising, but deterioration set in after some considerable time (Materia Medica Nordmark 16, [1964], page 245 and "Der Internist" 6 [1965] H. 5, page 216). Among the other disadvantages which were observed, for example, was that natural tissue did not grow into the synthetic fibre fabric. To overcome this disadvantage it has been proposed to make the synthetic fibre fabrics in a more open mesh, but this impaired other properties of the prostheses, for example, the strength thereof. A further disadvantage associated with the known synthetic fibre prostheses is the difficulty encountered in suturing the same into position because the synthetic fiber prostheses tear easily and the holes thus formed do not close.

The present invention overcomes the difficulties above mentioned and provides a prosthetic device for use in the replacement, repair and strengthening of living organs superior in effectiveness to anything previously known.

One of the objects of the invention is the provision of a prosthesis that is created from biological tissue which does not undergo deterioration after installation even after prolonged periods.

Another object is the provision of a prosthesis that is created from biological tissue that will allow for and facilitate tissue growth and organ regeneration at the site of installation.

## 2

A further object is the provision of a prosthesis that is created from biological tissue which can be simply and effectively installed using the conventional techniques.

Still a further object of the invention is the provision of a method by which such a prosthesis on a basis of biological tissue can be formed.

The manner in which these and other objects of this invention are obtained will become apparent from the detailed description and the following drawings in which:

10 FIG. 1 is a longitudinal central section through an embodiment of a prosthesis in accordance with the invention;

15 FIG. 2 is a diagrammatic view illustrating the method of forming the prosthesis of FIG. 1; and

20 FIGS. 3 and 4 are diagrammatic perspective views illustrating two somewhat different forms of the prostheses embodying the invention.

25 According to the invention there is provided a prosthesis in tubular, sheet or strip form which comprises at least two layers of biological tissue intimately joined and dried. More specifically the prosthesis comprises alternating layers of biological tissue and collagen fibers intimately joined and dried.

According to the present invention, the biological prostheses are manufactured by placing over, i.e., applying onto the surface of a firm support a piece of tubular, sheet or strip form biological tissue, causing the exposed surface thereof to swell so as to produce thereon an adhesive or glue like effect and/or the exposed surface is coated with 30 a binder or bonding agent as for example a collagen fiber paste, a second piece of biological tissue is then applied to the first and the procedure repeated until a multi-layered structure of the desired wall thickness is obtained. The prosthesis is then dried and removed from 35 the support.

As natural tissue for use in the manufacture of the prostheses of the invention there are suitable in particular the submucosa, which can be obtained in pure form from the small intestine of sheep, goats and other animals, 40 and the so-called "goldbeater's skin," which is made up of the serosa taken from the intestines of cattle. The submucosa, which is obtained in the form of a fine, but high strength tube, is composed of diagonally disposed collagen fibres. The mucosa and muscular tissue still adhering to 45 the submucosa can easily be removed by the process as conventionally used in the manufacture of catgut.

As the strength of a single layer of submucosa is far too inadequate, the same having a thickness of only about 15 $\mu$ , it is advantageous to use a number of layers 50 cemented together with a binder, as for example, a collagen fibre paste. The collagen fibre paste may be prepared, for example, by the process described in German patent specification No. 659,490. Furthermore, this layer of collagen fibres ensures that any holes, tears, 55 and the like made in the tissue during the manufacture thereof, during the operation for installing the same, or a later time, will close easily. This can prevent hemorrhage, which hitherto has been highly dangerous. The collagen fibre paste has a further advantage in that therapeutic substances may be incorporated therein. Thus, for 60 example, heparin may be added to inhibit the clotting of blood, cartilage powder or chondroitin sulfate included to stimulate the formation of new collagen fibres for the vascular intima, as well as other therapeutic substances.

65 It is also possible to cause the individual layers of tissue to swell and to bond them together in the swollen state. Organic acids, especially dilute lactic acid, have been found to be particularly suitable for swelling the single layers. The use of highly dilute solutions of lactic acid is preferred in this connection as the same has the advantage that no acidic end products are formed.

70 In carrying out the process of the invention it is

possible to use, for example, a tubular core or a plate made of glass or a synthetic material as the firm, more or less rigid support. Instances of synthetic materials include polyolefins as for example polyethylene or polypropylene etc. However, any inert fairly firm material may be employed. Prior to use, it is advantageous to treat the surface or surfaces of the support with a lubricant, as for example, glycerol or a silicone oil. A thoroughly cleansed tubular or flat piece of biological tissue, for example, submucosa or serosa tissue, which may have been subjected to bleaching with hydrogen peroxide, is then placed onto the support. The tissue is then coated with a binder paste, preferably a collagen fibre paste, and, if necessary, the paste is allowed to dry slightly. Another piece of tissue is then applied, and the process is repeated until the desired thickness is obtained. The finished prosthesis may contain, for example, about eight layers of tissue. The number of layers is generally determined by the thickness of the composite layers and by the ultimate use.

The prosthesis made by the process of the invention may be subjected to a hardening process to prevent premature absorption by the body tissues. As hardening agents there may be used physiologically acceptable vegetable or synthetic substances or, as for example, aldehydes. Instances of aldehydes that are suitable for this purpose are formaldehyde, glutardialdehyde and aldehydes of higher polyhydroxy compounds. The concentration of the hardening agent may be varied to produce the rate of absorption required.

The hardening process is preferably carried out after the final layer of tissue has been applied. However, it is possible to harden the single layers of tissue before they are applied. By adopting this latter procedure, the single layers of tissue may be hardened to varying degrees, thereby producing a prosthesis in which the single layers have different rates of absorption. For example, when using a tubular core as a support, the innermost layers may be hardened to a considerable degree to produce a tough, resistant core, and the outside layers may be only slightly hardened to ensure a specific rate of absorption.

After removal of the support and, if necessary, after the tube has been cut open, fascia prostheses are obtained which are generally known as "patches" and which may be used to close defects in the tympanic membrane and the heart wall, for hollow-walled organs or as heart valves.

Furthermore, collagen patches in sheet form are also used to repair damage to parenchymatous soft tissue, for example, in the liver, kidney, spleen and pancreas. This can be effected in the following manner:

A so-called mattress suture is made, i.e., a largeatraumatic needle threaded with a soft suture is passed through the parenchymatous tissue on one side of the wound and out of the other side. The needle is then passed through a stiffened and perforated collagen patch from underneath. The needle is then passed back through an adjacent perforation in the collagen patch at an appropriate distance from the point at which it emerged, through the organ and out the other side. The length of the suture should be such that a second perforated collagen patch may be threaded onto the two ends. When the needle has been removed, the two ends of the suture are knotted together over the collagen patch.

Strips for surgical purposes, as for example, for securing a movable kidney or for use in surgery of the incontinentia vesicae, may also be cut from sheets, i.e., membranes of the same material.

Tubular, flat or fluted prostheses may also be made by the process of the invention in addition to membranes and strips. The tubular prostheses may be of uniform diameter throughout their length or their diameter may be widened or narrowed conically.

Referring to the drawing a tube made of synthetic material as, for example, a tube made of polyethylene or

polypropylene and which has been provided with a plurality of threads 2 is thoroughly cleaned and, if necessary, treated with a silicone oil. A tube of tissue 3, preferably submucosa, which has been thoroughly cleansed and, if necessary, bleached with hydrogen peroxide, is drawn over the polyethylene tube 1, allowed to dry slightly, if necessary, and then a synthetic filament 4 is wound round the tubular tissue corresponding to the depressions of the thread and the tissue is dried. The filament may then be removed. The submucosa 3 is thus provided with a thread 2' and is of a standardized size. The tissue is then coated with a binder paste, preferably a collagen fibre paste, the paste is allowed to dry slightly, and then another tube of tissue is drawn over the first one. A synthetic filament is wound round it as before and the tissue is dried. This procedure may be repeated until the desired thickness of wall is obtained. The multiple layers of tissue are firmly cemented together by the binder. When the single layers of tissue are to be united by swelling it is possible either first to swell the single layers of tissue and to draw them onto the tube or core in the swollen state or to swell them on the core. To free the tube formed by these layers of tissue from the supporting tube or core, warm air is passed through the tube or core in this case a plastic tube, to soften it slightly, whereupon both ends of the tube are pulled until it stretches and detaches from the tissue at the beginning of the thread section. It can then be pulled out of the submucosa tube in the form of a plastic filament without the submucosa tube adhering to it or being damaged. Prostheses suitable for various purposes may be produced by varying the pitch of the thread, the depth of the thread and the number of turns.

The threaded tube of tissue so obtained has the necessary strength, density and elasticity required of vascular prostheses, and it can be sutured and is puncture-proof. The thread with which it is provided prevents it from kinking when it is moved after implantation in the host, thereby permitting an unhindered flow of blood. It is also extensible.

On the other hand, if a smooth tubular prosthesis is required, that is to say, without any thread or fluting, for example, as used for prosthetic repair of the cystic duct, the ureter, the esophagus or, in special cases, blood vessels, the same procedure as with the screw-threaded plastic tube may be followed, but without winding a filament round the tissue or allowing it to conform to the shape of the thread. The elastic tube of tissue is drawn over the plastic tube and held taut over it by tying the tissue tube at both ends and allowing it to conform to the outer circumference of the plastic tube without complementing the shape of the thread. Alternatively, a smooth plastic tube may be used as a support, for the layers of tissue.

Prostheses, for example, for the esophagus, trachea and intestine, can be made by the process described above, with due regard to anatomical requirements, diameter and thickness of wall. The strength of such prostheses can be considerably increased by placing layers of synthetic or natural tissue or even metallic clasps or spirals between the layers making up the actual prosthesis. The synthetic tissue used may be made, for example, from polyamide or polyester fibres. The natural tissue may be, for example, biological tissue, for example, serosa tissue, or material made from natural fibres. The serosa tissue may be wound round the prosthesis diagonally, first from left to right and then from right to left. If necessary, these layers of tissue may be pre-treated, as for example, by stretching.

It is also possible to bond the layers of tissue by swelling the tubular or flat pieces in an acidic or alkaline medium. In this process the upper layers of collagen fibers are slightly hydrolyzed and converted into tropocollagen which, on drying, has a glue-like adhesive effect.

The process has a negative effect on the physical properties of the collagen fibre and neutralization is generally necessary afterwards, followed by washing out of the salts formed during neutralization.

Sterilization of the prostheses so obtained may be effected by gamma-radiation, which process also reduces the antigenic properties of the collagen.

In FIGS. 3 and 4 there are shown two somewhat different forms of the prostheses in accordance with the invention. In FIG. 3 the embodiment comprising alternating layers of biological tissue 7 bonded together with a bonding agent 8 is shown and in FIG. 4 the embodiment wherein the bonding is effected by swelling the layers 7 is set out.

The prostheses in accordance with the invention has been subjected to trial and has been observed and evaluated as a suitability, production of toxic symptoms, decomposition, detachment, secondary reactions such as abnormal tissue growth, etc. The trials consisted in surgical implantation of the prostheses in otherwise normal animals, i.e., the requirement for the prostheses was surgically induced, observation of the thusly treated animals during the recovery period and for varying periods thereafter. During this time, numerous test procedures were carried out, the same including chemical, X-ray, electrocardiographic, etc., procedures. At the end of various predetermined time intervals certain of the animals were sacrificed and any of the animal's possibly involved organs examined both microscopically and macroscopically. In every instance, the results of procedures and tests in both the living and sacrificed animals established the safety and suitability of the prosthetic devices for replacement and repair of damaged organs. It is to be noted that as experimental animals, there were employed cats, dogs and monkeys.

The device has been surgically implanted in human subjects, in each case where the subject's condition was indicative of such treatment. Almost all of the subjects are still under observation and to date there have not been observed any untoward results or happenings directly associated with the use of the herein disclosed prosthetic devices.

What is claimed is:

1. A tubular prosthetic device on a basis of biological tissue comprising at least two superimposed layers consisting of tubes of natural tissue applied in their natural tubular form prepared from the submucous layers of intestines of mammals, and said layers being bonded together by means of collagen fibers.

2. A prosthetic device according to claim 1 wherein said collagen fibres consist of a collagen fiber paste.

3. A prosthetic device according to claim 1 wherein at least one of said layers is a prehardened layer which has been prehardened by contacting the same with a hardening agent.

4. A prosthetic device according to claim 3 wherein said hardening agent is an aldehyde.

5. A hardened prosthetic device according to claim 1 wherein said prosthetic device has been hardened by treatment thereof with a hardening agent.

20

#### References Cited

##### UNITED STATES PATENTS

|           |        |                |       |           |
|-----------|--------|----------------|-------|-----------|
| 1,254,031 | 1/1918 | Davis          | ----- | 128—335.5 |
| 2,127,903 | 8/1938 | Bowen          | ----- | 128—334   |
| 3,272,204 | 9/1966 | Artandi et al. | ----- | 128—334   |
| 3,366,440 | 1/1968 | Nuwayser       | ----- | 128—334X  |
| 3,425,418 | 2/1969 | Chvapil et al. | ----- | 128—334   |

##### OTHER REFERENCES

30 "Experimental and Clinical Utilization of a Prosthesis for Replacement of the Trachea," by R. E. Taber et al., A.M.A. Archives of Surgery, vol. 77, October 1958, pp. 576—583.

35 DALTON L. TRULUCK, Primary Examiner

R. L. FRINKS, Assistant Examiner

U.S. Cl. X.R.

40 128—334; 156—326, 83, 307; 8—94.11, 94.18